

## 1

3,390,080

**MOLYBDENUM DISULPHIDE**

Aleksander Jerzy Groszek, Ealing, London, England, assignor to The British Petroleum Company Limited, London, England, a corporation of Great Britain  
No Drawing. Filed Sept. 21, 1966, Ser. No. 586,346  
Claims priority, application Great Britain, Sept. 24, 1965,

40,700/65

6 Claims. (Cl. 252—25)

This invention relates to a novel molybdenum disulphide product of a particular physical form in which it possesses new and useful properties.

It is well known to grind molybdenum disulphide in air using, for example, rotary or vibratory ball mills. The finely-divided molybdenum disulphide can be used either by itself as a dry, solid lubricant or in dispersions with lubricating properties.

According to the invention, a novel molybdenum disulphide, with a surface area (as determined by nitrogen adsorption) of from 10 to 400 square metres per gram, is provided which is prepared by grinding the molybdenum disulphide in a low boiling point, low viscosity, low surface tension organic liquid. For convenience, the disulphide product prepared in this way will hereinafter be called "oleophilic" molybdenum disulphide to distinguish it from the untreated starting material. "Oleophilic" molybdenum disulphide has a considerable tendency to adsorb n-dotriacontane in preference to n-butanol (1), in contrast to the untreated starting material.

The molybdenum disulphide used may be either natural or artificial. One example of a natural molybdenum disulphide product is that supplied by Acheson Colloids, "Dag 325."

Satisfactory products can be obtained by grinding in most organic liquids, but it is desirable to use one, the bulk of which can be easily removed from the oleophilic molybdenum disulphide. Those liquids distilling below 500° C. and having a viscosity below 600 centistokes at 100° F. (38° C.) are therefore preferred. Liquids having a surface tension below 72 dynes/cm., preferably from 10 to 40 dynes/cm., at 25° C. are preferred.

Suitable organic liquids are lower molecular weight hydrocarbons, including straight-chain or branched-chain, saturated or unsaturated alkyls, saturated or unsaturated, substituted or unsubstituted, cycloalkyls, and substituted or unsubstituted aromatic compounds. Examples of such compounds are n-heptane, octene-2, 2,2,4-trimethylpentane, cyclohexane, benzene or toluene. Branched alkyl compounds are particularly preferred. Other suitable organic liquids are those compounds which contain fluorine, chlorine, or phosphorus and chlorine, for example, carbon tetrachloride.

Other suitable organic liquids are the polar oxygen compounds such as isopropyl alcohol. Silicone fluids can also be used.

For best results, the amount of molybdenum disulphide in the molybdenum disulphide/organic liquid mixture should not exceed 50% wt., preferably it should be from 2 to 20% wt.

The grinding may be carried out in any suitable grind-

## 2

ing mill or device and it is desirable to continue the grinding until an oleophilic molybdenum disulphide having a surface area (as determined by nitrogen adsorption) of from 10 to 400, preferably from 30 to 200, square metres per gram is obtained. Usually this can be achieved by grinding at normal temperatures for the required period but the temperature of the mixture may be artificially increased if desired, for example, up to 400° C. In this case, liquids which have viscosities up to 600 centistokes at 100° F. (38° C.) may be used, for example, mineral lubricating oils, ranging from "spindle" oils to "bright stocks."

One of the quickest and most effective techniques is to carry out the grinding in a vibratory ball mill.

It is desirable to exclude air so far as possible during the grinding operation and this can be most easily achieved by filling the mill with the organic liquid first, followed by the balls and molybdenum disulphide. A suitable procedure is to fill the mill with the liquid, add half the balls, then the molybdenum disulphide and finally the rest of the balls.

When using a ball mill, it is of course desirable to use balls made of a material which does not react with the graphite and which does not wear unduly the grinding. Vibratory ball mills usually contain steel balls and these are suitable for the present purpose. It is preferred to use a hard grade of steel for the balls.

A magnetic filter can be used to remove small steel particles from the slurry. A circulatory system can also be used wherein the slurry is pumped through an internal magnetic filter and then returned to the mill.

A suitable vibratory ball mill is sold under the trade name "Megapact" (2), manufactured by Pilamec Limited. The grinding effect is produced by the impact of the balls upon the molybdenum disulphide and upon each other.

The slurry of oleophilic molybdenum disulphide can be separated from the balls by sieving or by displacement by another liquid and sieving.

If a relatively high boiling organic liquid is used for grinding it is preferred to displace this liquid by a low boiling liquid. This liquid can then be removed by boiling. It is preferred to use vigorous boiling.

It is also possible to filter the slurry to obtain a filter cake of oleophilic molybdenum disulphide.

In either case it is preferred to remove the last traces of solvent by heating the filter cake in a vacuum oven for several hours, for example, at 100° C. and at 1 mm. mercury.

The following examples serve to illustrate the invention.

**Example 1**

Two oleophilic molybdenum disulphide products according to the invention were prepared from commercial disulphides. The table below compares the properties of commercial, non-oleophilic molybdenum disulphides.

It is thought that the proportions of surface area of the disulphide with "polar" sites or with "non-polar" sites are measured by the heats of adsorption of n-butanol or n-dotriacontane and that the ratios of heats of adsorption gives same measure of the ratios of "polar" to "non-polar" sites.

(1) See notes at end of specification.

(2) See notes at end of specification.

| Reference No. | Type of MoS <sub>2</sub>                                                           | BET Surface Area, metre <sup>2</sup> /gram | Heat of Adsorption of n-butanol in millicalories/gram | Heat of Adsorption of n-C <sub>32</sub> in millicalories/gram |
|---------------|------------------------------------------------------------------------------------|--------------------------------------------|-------------------------------------------------------|---------------------------------------------------------------|
| Example A     | Commercial MoS <sub>2</sub> "A" ground in n-heptane for 4 hours ("Megapact" mill). | 40                                         | 384                                                   | 396                                                           |
| Example B     | Commercial MoS <sub>2</sub> "B" ground in n-heptane for 4 hours ("Megapact").      | 39                                         | 380                                                   | 470                                                           |
| Comparison 1  | Commercial MoS <sub>2</sub> "A" ground in air for 4 hours ("Megapact").            | 65                                         | 1,400                                                 | 335                                                           |
| Comparison 2  | Commercial MoS <sub>2</sub> "B" (as obtained from maker).                          | 5                                          | 42                                                    | 9.6                                                           |
| Comparison 3  | Commercial MoS <sub>2</sub> "C" (as obtained from maker).                          | 8                                          | 281                                                   | 110                                                           |
| Comparison 4  | Commercial MoS <sub>2</sub> "A" ground by makers.                                  | 22                                         |                                                       |                                                               |

The comparison samples 1 and 4 show some oleophilic properties, but they do, however, adsorb n-butanol to a large extent. Although the oleophilic molybdenum disulphides used in Examples A and B adsorb n-butanol they have very much higher ratios than do comparison samples 1 and 4.

The materials produced in Examples A and B can be used as thickeners of organic fluids, which form the base oils, to form dispersions or infusible greases. The greases show good mechanical stability. This use of the oleophilic molybdenum disulphide forms the subject of our co-pending U.S. patent application Ser. No. 580,868 filed Sept. 21, 1966. The oleophilic molybdenum disulphides can also be used as adsorbents for waxy components of petroleum distillates and their dewaxing activity is rather more selective towards waxes than is the case with other molybdenum disulphides. This use of the oleophilic molybdenum disulphide forms the subject of our co-pending U.K. patent application No. 33,531/65.

#### Example 2

It was found that the particle shape of oleophilic molybdenum disulphides was considerably different to the particle shape of air-ground molybdenum disulphides. Oleophilic molybdenum disulphides comprised thin, plate-like particles with major dimensions from 0.1 to 5 microns by from 0.1 to 5 microns and from 50 to 200 angstroms thick. On the other hand air-ground molybdenum disulphides comprised chunky particles with dimensions ranging from 0.1 x 0.1 x 0.1 micron to 0.5 x 0.5 x 0.5 micron.

#### NOTES

(1) The heats of adsorption of n-dotriacontane and n-butanol on the molybdenum disulphide were measured using the Flow Microcalorimeter as described in Chemistry and Industry, Mar. 20, 1965, 482-489.

(2) The "Megapact" mill contains grinding chambers which are steel cylinders of 1 1/4-inch interior diameter by 15 inches long and which are nearly filled with 1/4 inch diameter steel balls. The mill is fitted with a one-eighth horsepower electric motor and the oscillation can

be adjusted from 1 to 5 mm. In operation, each cylinder was filled completely with the n-heptane and the steel balls and 25 to 30 grams of molybdenum disulphide were added. This left from 150 to 200 cc. n-heptane in each cylinder. The ends of the cylinders were then sealed by metal caps fitted with rubber washers and the grinding carried out. After grinding, the contents of the cylinders were placed in sieves which retained the balls and the n-heptane was removed from the oleophilic molybdenum disulphide by evaporation.

I claim:

1. An oleophilic molybdenum disulphide with a surface area of from 10 to 400 square metres per gram, prepared by grinding natural or synthetic molybdenum disulphide in organic liquid distilling below 500° C., having a viscosity below 600 centistokes at 38° C. and a surface tension less than 72 degrees/cm. at 25° C.
2. A product as claimed in claim 1, wherein the organic liquid has a surface tension from 10 to 40 dynes/cm. at 25° C.
3. A product as claimed in claim 1, wherein the grinding is carried out in a vibratory ball mill.
4. A product as claimed in claim 1, wherein the amount of molybdenum disulphide in the molybdenum disulphide/organic liquid mixture does not exceed 50% wt., based on the weight of mixture.
5. A product as claimed in claim 1, wherein the amount of molybdenum disulphide in the molybdenum disulphide/organic liquid mixture is from 2 to 20% wt.
6. A product as claimed in claim 1, wherein the surface area of the molybdenum disulphide is from 30 to 200 square metres per gram.

#### References Cited

##### UNITED STATES PATENTS

- |           |         |         |        |
|-----------|---------|---------|--------|
| 3,059,769 | 10/1962 | Frost   | 252-25 |
| 3,338,822 | 8/1967  | Groszek | 252-25 |

DANIEL E. WYMAN, Primary Examiner.

I. VAUGHN, Assistant Examiner.

UNITED STATES PATENT OFFICE  
CERTIFICATE OF CORRECTION

Patent No. 3,390,080

June 25, 1968

Aleksander Jerzy Groszek

It is certified that error appears in the above identified patent and that said Letters Patent are hereby corrected as shown below:

Column 4, line 29, "72 degrees/cm. at 25° C" should read  
-- 72 dynes/cm. at 25° C --.

Signed and sealed this 9th day of December 1969.

(SEAL)

Attest:

Edward M. Fletcher, Jr.

Attesting Officer

WILLIAM E. SCHUYLER, JR.

Commissioner of Patents